



US007759429B2

(12) **United States Patent**  
**Kowaki et al.**

(10) **Patent No.:** **US 7,759,429 B2**  
(45) **Date of Patent:** **\*Jul. 20, 2010**

(54) **FLAME-RETARDANT POLYESTER FIBERS  
FOR ARTIFICIAL HAIR**

(75) Inventors: **Toshihiro Kowaki**, Osaka (JP);  
**Toshiyuki Masuda**, Hyogo (JP);  
**Hiroyuki Shinbayashi**, Osaka (JP);  
**Toyohiko Shiga**, Hyogo (JP)

(73) Assignee: **Kaneka Corporation**, Osaka-shi (JP)

(\*) Notice: Subject to any disclaimer, the term of this patent is extended or adjusted under 35 U.S.C. 154(b) by 961 days.

This patent is subject to a terminal disclaimer.

(21) Appl. No.: **10/565,744**

(22) PCT Filed: **Jul. 25, 2004**

(86) PCT No.: **PCT/JP2004/010740**

§ 371 (c)(1),  
(2), (4) Date: **Jan. 23, 2006**

(87) PCT Pub. No.: **WO2005/010247**

PCT Pub. Date: **Feb. 3, 2005**

(65) **Prior Publication Data**

US 2006/0194044 A1 Aug. 31, 2006

(30) **Foreign Application Priority Data**

Jul. 25, 2003 (JP) ..... 2003-201875  
Oct. 17, 2003 (JP) ..... 2003-358314  
Dec. 5, 2003 (JP) ..... 2003-408325  
Mar. 19, 2004 (JP) ..... 2004-081033

(51) **Int. Cl.**

**A41G 5/00** (2006.01)  
**C08L 77/00** (2006.01)  
**C08L 67/00** (2006.01)  
**D01F 11/08** (2006.01)

(52) **U.S. Cl.** ..... **525/397; 525/408; 525/438;**  
**524/371; 428/364; 428/397; 428/400; 428/401;**  
**132/201; 8/529; 8/532**

(58) **Field of Classification Search** ..... **525/438;**  
**57/253; 132/201; 8/529-534**  
See application file for complete search history.

(56) **References Cited**

**U.S. PATENT DOCUMENTS**

4,506,043 A \* 3/1985 Ogawa et al. ..... 523/523  
(Continued)

**FOREIGN PATENT DOCUMENTS**

CN 1075131 C 12/1996  
(Continued)

**OTHER PUBLICATIONS**

International Search Report from Corresponding International Application No. PCT/JP2004/010740, dated Nov. 22, 2004, 4 pages.  
(Continued)

*Primary Examiner*—Randy Gulakowski

*Assistant Examiner*—Mike Dollinger

(74) *Attorney, Agent, or Firm*—Westerman, Hattori, Daniels & Adrian, LLP

(57) **ABSTRACT**

A flame retardant polyester fiber for artificial hair, which is obtained by melt spinning a composition as a mixture of 100 parts by weight of (A) a polyester made of one or more of polyalkylene terephthalate and a copolymer polyester comprising polyalkylene terephthalate as a main component with 5 to 30 parts by weight of (B) a brominated epoxy flame retardant. The present invention also relates to the polyester fiber for artificial hair which has at least one modified cross-section, is a mixture with a fiber having a modified cross-section, and has a mixing ratio of the fiber having a round cross-section to the fiber having a modified cross-section is 8:2 to 1:9, and to the flame retardant polyester fiber for artificial hair which further comprises a hydrophilic fiber treating agent attached thereto, and thus has excellent smooth feeling, combing properties, and flame retardance.

**21 Claims, 4 Drawing Sheets**



## U.S. PATENT DOCUMENTS

|                 |         |                      |           |
|-----------------|---------|----------------------|-----------|
| 4,525,404 A *   | 6/1985  | Matsui et al. ....   | 428/92    |
| 4,562,216 A *   | 12/1985 | Kishida et al. ....  | 523/433   |
| 4,732,921 A *   | 3/1988  | Hochberg et al. .... | 523/460   |
| 5,083,967 A *   | 1/1992  | Yokoe et al. ....    | 446/394   |
| 5,614,568 A *   | 3/1997  | Mawatari et al. .... | 523/122   |
| 5,954,062 A     | 9/1999  | Murata               |           |
| 7,332,563 B2 *  | 2/2008  | Masuda et al. ....   | 528/308.1 |
| 7,501,463 B2 *  | 3/2009  | Kowaki et al. ....   | 524/109   |
| 2006/0154062 A1 | 7/2006  | Kowaki et al.        |           |

## FOREIGN PATENT DOCUMENTS

|    |             |        |
|----|-------------|--------|
| CN | 1221583     | 7/1999 |
| CN | 1337489     | 2/2002 |
| JP | 48-13277    | 2/1973 |
| JP | 60-071713 A | 4/1985 |
| JP | 62-170519 A | 7/1987 |
| JP | 3-124761 A  | 5/1991 |

|    |                  |         |
|----|------------------|---------|
| JP | 5-86505 A        | 4/1993  |
| JP | 8-19568 B2       | 2/1996  |
| KR | 1982-0001211 B1  | 7/1982  |
| KR | 1998-084288      | 12/1998 |
| KR | 1999-0040635     | 6/1999  |
| KR | 10-0215251 B1    | 8/1999  |
| KR | 2004-61347       | 7/2004  |
| WO | WO 03071014 A1 * | 8/2003  |

## OTHER PUBLICATIONS

International Preliminary Report on Patentability (Chapter I of the Patent Cooperation Treaty) from Corresponding International Application No. PCT/JP2004/010740, dated May 22, 2006, 7 pages.

“Studies on New Hydrophilic Finishing Agent for Fabrics,” Journal of Qiqiha’er Institute of Light Industry, vol. 4, Aug. 31, 1988, 11 pages. (Partial Translation).

The Office Action for Corresponding Chinese Patent Application No. 2004800210767 dated Aug. 17, 2007, 5 pages.

\* cited by examiner



FIG.1



FIG.2



FIG.3

FIG.4



FIG.5



FIG.6





FIG.7



FIG.8



FIG.9



FIG.10

## FLAME-RETARDANT POLYESTER FIBERS FOR ARTIFICIAL HAIR

### RELATED APPLICATIONS

This application is a nationalization of PCT application PCT/JP2004/010740 filed on Jul. 20, 2004, claiming priority based on Japanese Patent Application No. 2003-201875 (Jul. 25, 2003), Japanese Patent Application No. 2003-358314 (Oct. 17, 2003), Japanese Patent Application No. 2003-408325 (Dec. 5, 2003) and Japanese Patent Application No. 2004-081033 (Mar. 19, 2004), the contents of which are incorporated herein by reference in their entirety.

### TECHNICAL FIELD

The present invention relates to a flame retardant polyester fiber for artificial hair, made of a polyester and a brominated epoxy flame retardant. More particularly, the present invention relates to a fiber for artificial hair which maintains fiber properties such as flame resistance, heat resistance, and strength and elongation, and has excellent curl-setting properties, transparency, devitrification resistance, and combing properties.

The present invention also relates to a modified cross-section fiber. More particularly, the present invention relates to a modified cross-section fiber having luster, hue, texture and bulkiness close to human hair, which is used as a fiber for artificial hair for hair goods or the like such as wig, braid, or extension hair, and to a fiber for artificial hair using the modified cross-section fiber.

Furthermore, the present invention relates to a fiber for artificial hair which has excellent smooth feeling, combing properties, and antistatic properties.

### BACKGROUND ART

Fibers made of polyethylene terephthalate or a polyester comprising polyethylene terephthalate as a main component has excellent heat resistance, chemical resistance, a high melting point and a high modulus of elasticity, therefore are thus widely used in curtains, carpets, clothes, blankets, sheetings, table clothes, upholstery fabrics, wall coverings, artificial hair, interior materials for automobiles, outdoor reinforcing materials, and safety nets.

On the other hand, human hair, artificial hair (modacrylic fibers, polyvinyl chloride fibers), or the like has been conventionally used in hair products such as wigs, hair wigs, extensions, hair bands, and doll hair. However, it has now become difficult to provide human hair for hair products, and thus artificial hair has become more important. Modacrylic fibers have been often used as artificial hair materials due to their flame retardance, but have only insufficient heat resistance.

In recent years, there has been proposed artificial hair using, as a main component, a polyester typified by polyethylene terephthalate having excellent heat resistance. However, fibers made of a polyester typified by polyethylene terephthalate are flammable materials, and thus have insufficient flame resistance.

Conventionally, various attempts have been made to improve flame resistance of polyester fibers. Known examples of such attempts include a method comprising using a fiber made of a polyester obtained by copolymerizing a flame retardant monomer containing a phosphorus atom, and a method comprising adding a flame retardant to a polyester fiber.

As the former method comprising copolymerizing a flame retardant monomer, a method comprising copolymerizing a phosphorus compound with excellent heat stability having a phosphorus atom as a ring member (Japanese Patent Publication No. 55-41610), a method comprising copolymerizing carboxyphosphinic acid (Japanese Patent Publication No. 53-13479), a method comprising copolymerizing a polyester containing a polyallylate with a phosphorus compound (Japanese Patent Laid-open No. 11-124732), or the like has been proposed.

As artificial hair to which the above flame retardant technology is applied, a polyester fiber copolymerized with a phosphorus compound has been proposed (Japanese Patent Laid-open No. 03-27105, Japanese Patent Laid-open No. 05-339805, etc.), for example.

However, since artificial hair is demanded to be highly flame resistant, such a copolymer polyester fiber must have a high copolymerization amount when used for artificial hair. This results in a significant decrease in flame resistance of the polyester, and causes other problems in which it is difficult to perform melt spinning, or, when flame approaches, the artificial hair does not catch fire and is not burned, but molten and dripped. When the phosphorus flame retardant is added, stickiness is increased because it must be added in a large amount to exhibit flame retardance, and the resulting artificial hair made of a polyester fiber tends to have a heat history and, under high humidity conditions, be devitrified to affect the appearance of the fiber.

On the other hand, as the latter method comprising adding a flame retardant, a method comprising adding a halogenated cycloalkane compound as fine particles to a polyester fiber (Japanese Patent Publication No. 03-57990), a method comprising adding a bromine-containing alkylcyclohexane to a polyester fiber (Japanese Patent Publication No. 01-24913), or the like has been proposed. However, in the method comprising adding a flame retardant to a polyester fiber, in order to achieve sufficient flame retardance, the addition treatment temperature must be as high as 150° C. or more, the addition treatment time must be long, or a large amount of a flame retardant must be used, disadvantageously. This causes problems such as deteriorated fiber properties, reduced productivity, and an increased production cost.

As described above, artificial hair has not yet been provided which maintains fiber properties possessed by a conventional polyester fiber such as flame resistance, heat resistance, and strength and elongation and has excellent setting properties, devitrification resistance, and stickiness reduction.

Synthetic fibers conventionally used for hair include acrylonitrile fibers, vinyl chloride fibers, vinylidene chloride fibers, polyester fibers, nylon fibers, and polyolefin fibers. Conventionally, these fibers have been processed into products for artificial hair such as wigs, braids, and extension hair. However, these fibers do not have properties necessary for a fiber for artificial hair such as heat resistance, curling properties, and good feeling together. Thus, products with various properties satisfied cannot be produced from a single fiber, and products making use of properties of each fiber are produced and used. Fibers having a cross-section suitable to characteristics of each goods have also been studied and improved.

Examples of such fibers include a filament for wigs having a cocoon cross-section with a length L of a longest part, a diameter W of round parts on both ends, and a width C of a central constriction, each within a specific range (Japanese Utility Model Laid-open No. 48-13277); a synthetic fiber for artificial hair having a largest diameter (L) passing through

the gravity in the fiber cross-section within a specific range (Japanese Patent Publication No. 53-6253); a filament for wigs and braids having a Y-shaped cross-section in which four unit filaments having an almost round shape or an elliptical shape are provided with one unit filament radially adjacent to the other three unit filaments at the same intervals, and the adjacent unit filaments have contact points having a width almost equal to the radius of the unit filaments (Japanese Utility Model Laid-open No. 63-78026); and a filament for wigs having a cross-section with at least two flat circles lapped, in which the ratio L/W of the major axis length L to the minor axis length W, the distance between the centers of two adjacent flat circles, the angle between the straight line linking the centers of two adjacent flat circles and the major axes of the flat circles, and the like are limited (Japanese Patent Laid-open No. 55-51802).

However, any of the above-described conventional fibers developed as fibers for artificial hair has a cross-section with a length and an angle extremely limited and with a unique shape, and cannot necessarily easily produced. In addition, such fibers do not necessarily have preferable texture when used for braids or extension hair, and tend to be felt hard because the fibers are intended to keep a hairstyle or make the resulting hair straight. Further, these fibers cannot be sufficiently easily handled manually. Ribbon-section fibers have conventionally widely used for piles, but have been assumed to be inappropriate for use as fibers for artificial hair such as wigs due to their disliked too much softness or the like.

On the other hand, in the method comprising adding a flame retardant to a polyester fiber, in order to achieve sufficient flame retardance, the addition treatment temperature must be as high as 150° C. or higher, the addition treatment time must be long, or a large amount of a flame retardant must be used, disadvantageously. This causes problems such as deteriorated fiber properties, decreased productivity, and an increased production cost.

In order to provide such synthetic fibers poorly flame retardant or not flame retardant with flexibility, smooth feeling, or the like, various silicone finishing agents have been provided. Examples of the finishing agents for providing the fibers with flexibility, crease resistance, elastic force, and compression recovery properties include dimethylpolysiloxane, methylhydrogenpolysiloxane, dimethylpolysiloxane having hydroxyl groups at both terminals, a vinyl group-containing organopolysiloxane, an epoxy group-containing organopolysiloxane, an amino group-containing organopolysiloxane, an ester group-containing organopolysiloxane, and a polyoxalkylene-containing organopolysiloxane. A treating agent composed of a combination of alkoxy silanes and/or a polyacrylamide resin or a catalyst or the like has also been known.

For example, there is disclosed a method using a treating agent composed of an organopolysiloxane containing at least two epoxy groups in one molecule and an organopolysiloxane containing an amino group, or a treating agent composed of an organopolysiloxane having hydroxyl groups at both terminals, and an organopolysiloxane containing an amino group and an alkoxy group in one molecule and/or its partial hydrolysate and condensate (Japanese Patent Publication No. 53-36079).

Further, there are described a treating agent composed of an organopolysiloxane containing an epoxy group and an aminoalkyltrialkoxysilane (Japanese Patent Publication No. 53-197159 and Japanese Patent Publication No. 53-19716), and a diorganopolysiloxane having triorganosiloxy groups at both terminals, which contains two or more amino groups in one molecule (Japanese Patent Publication No. 53-98499). In

addition, there is proposed a method using a treating agent composed of an aminopolysiloxane containing two or more amino groups in one molecule and an alkoxy silane containing one or more reactive groups such as amino groups or epoxy groups (Japanese Patent Publication No. 58-17310).

Further, there are disclosed a method using a treating agent composed of a diorganopolysiloxane containing at least two amino groups in one molecule and a diorganopolysiloxane containing at least two ester bonds in one molecule (Japanese Patent Laid-open No. 55-152864), and a method using a polysiloxane containing an amino group, a hydroxyl group-terminated polysiloxane, and an alkylalkoxysilane containing a reactive group (Japanese Patent Laid-open No. 58-214585). In addition, there are disclosed a method using a treating agent composed of an organopolysiloxane containing an epoxy group, an aminosilane compound, and a curing catalyst (Japanese Patent Laid-open No. 59-144683), and a method using an organopolysiloxane containing at least two epoxy groups in one molecule and a polyacrylamide resin (Japanese Patent Laid-open No. 60-94680).

However, fibers to which these silicone-containing fiber treating agents are attached exhibit improved smooth feeling, combing properties, and the like, but the silicone-containing fiber treating agents are flammable, and thus provide significantly reduce flame retardance of flame retardant synthetic fibers, disadvantageously.

#### DISCLOSURE OF THE INVENTION

The present invention relates to a flame retardant polyester fiber for artificial hair, formed from 100 parts by weight of (A) a polyester made of one or more of polyalkylene terephthalate and a copolymer polyester comprising polyalkylene terephthalate as a main component, and 5 to 30 parts by weight of (B) a brominated epoxy flame retardant represented by the general formula (1):



and more preferably the flame retardant polyester fiber for artificial hair, wherein the component (A) is a polyester made of at least one polymer selected from the group consisting of polyethylene terephthalate, polypropylene terephthalate, and polybutylene terephthalate, or the flame retardant polyester fiber for artificial hair, wherein the component (B) is at least one flame retardant selected from the group consisting of brominated epoxy flame retardants represented by the general formulas (α) to (γ):



wherein p represents 0 to 150, and y represents 0 to 5.

Preferably, the present invention relates to the flame retardant polyester fiber for artificial hair, characterized by comprising the components (A) and (B) further mixed with (C) organic fine particles and/or (D) inorganic fine particles to form minute projections on the fiber surface, wherein the component (C) is at least one member selected from the group consisting of a polyallylate, polyamide, fluororesin, silicone resin, crosslinked acrylic resin, and crosslinked polystyrene, or wherein the component (D) is at least one member selected from the group consisting of calcium carbonate, silicon oxide, titanium oxide, aluminum oxide, zinc oxide, talc, kaolin, montmorillonite, bentonite, mica, and an antimony compound.

The present invention also relates to a fiber for artificial hair, comprising the flame retardant polyester fiber to which (E) a hydrophilic fiber treating agent comprising an aliphatic polyether compound as a main component is attached. A flame retardant fiber for artificial hair is thus provided which does not have reduced flame retardance as in the case where a flame retardant polyester fiber, a flame retardant polypropylene fiber, a flame retardant polyamide fiber, or the like is treated with a silicone fiber treating agent in order to improve smooth feeling and texture, for example; has slip feeling, combing properties, and antistatic properties the same as in the case where such a fiber is treated with a silicone oil agent for the same purpose; and has excellent flame retardance.

Further, the polyester fiber of the present invention can have a specific modified cross-section. The present invention further relates to the polyester fiber for artificial hair, which has at least one modified cross-section selected from the group consisting of shapes of an ellipse, crossed circles, a cocoon, a potbelly, a dog bone, a ribbon, three to eight leaves, and a star. The present invention also relates to the polyester fiber for artificial hair, wherein the fiber cross-section has a shape with two or more circles or flat circles lapped or brought into contact with each other. The present invention also relates to the polyester fiber for artificial hair, wherein the fiber cross-section has a shape of three to eight leaves, and the fiber is a modified cross-section fiber having a degree of modification represented by the expression (1) of 1.1 to 8. The present invention further relates to the polyester fiber for artificial hair, wherein the fiber cross-section has a flatness ratio of 1.2 to 4. The present invention still further relates to the polyester fiber for artificial hair, which is a mixture of a fiber having a round cross-section with a fiber having at least one modified cross-section selected from the group consisting of shapes of an ellipse, crossed circles, a cocoon, a potbelly, a dog bone, a ribbon, three to eight leaves, and a star, wherein the mixing ratio of the fiber having a round cross-section to the fiber having a modified cross-section is 8:2 to 1:9.

Preferably, the flame retardant polyester fiber for artificial hair is in the form of a non-crimped fiber, is spun dyed, and has a monofilament size of 30 to 80 dtex.

## BRIEF DESCRIPTION OF THE DRAWINGS

FIGS. 1 to 10 are schematic views respectively showing a cross-section of a polyester fiber made of the composition of the present invention, with the figures corresponding to the following:

FIG. 1: A view of a cross-section in the shape of crossed circles

FIG. 2: A view of a cross-section in the shape of crossed flat circles

FIG. 3: A view of a cross-section in the shape of a dog bone

FIG. 4: A view of a cross-section in the shape of three leaves

FIG. 5: A view of a cross-section in the shape of five leaves

FIG. 6: A view of a cross-section in the shape of seven leaves

FIG. 7: A view for describing a flatness ratio of a modified cross-section

FIG. 8: A modified nozzle 1

FIG. 9: A modified nozzle 2

FIG. 10: A modified nozzle 3

## BEST MODE FOR CARRYING OUT THE INVENTION

The flame retardant polyester fiber for artificial hair of the present invention is a fiber obtained by melt spinning a composition comprising (A) a polyester made of one or more of polyalkylene terephthalate or a copolymer polyester comprising polyalkylene terephthalate as a main component, and (B) a brominated epoxy flame retardant. Examples of the polyalkylene terephthalate or the copolymer polyester comprising polyalkylene terephthalate as a main component, which is contained in the polyester (A) used in the present invention, include polyalkylene terephthalates such as polyethylene terephthalate, polypropylene terephthalate, and polybutylene terephthalate, and/or a copolymer polyester comprising such polyalkylene terephthalate as a main component and a small amount of a copolymerization component. The phrase "containing as a main component" refers to "containing in an amount of 80 mol % or more".

Examples of the copolymerization component include polycarboxylic acids such as isophthalic acid, orthophthalic acid, naphthalenedicarboxylic acid, paraphenylenedicarboxylic acid, trimellitic acid, pyromellitic acid, succinic acid, glutaric acid, adipic acid, suberic acid, azelaic acid, sebacic acid, and dodecanedioic acid, and their derivatives; 5-sodiumsulfoisophthalic acid; dicarboxylic acids including sulfonic acid salts such as dihydroxyethyl 5-sodiumsulfoisophthalate, and their derivatives; 1,2-propanediol, 1,3-propanediol, 1,4-butanediol, 1,6-hexanediol, neopentyl glycol, 1,4-cyclohexanediethanol, diethylene glycol, polyethylene glycol, trimethylolpropane, pentaerythritol, 4-hydroxybenzoic acid, and  $\epsilon$ -caprolactone.

Typically, the copolymer polyester is preferably produced by adding a small amount of a copolymerization component to a main component which is a polymer of terephthalic acid and/or its derivative (for example, methyl terephthalate) and alkylene glycol, and reacting these components, in view of stability and convenience for handling. However, the copolymer polyester may be produced by adding a small amount of a monomer or oligomer component as a copolymerization component to a main component which is a mixture of terephthalic acid and/or its derivative (for example, methyl terephthalate) and alkylene glycol, and polymerizing the components.

The copolymer polyester may be any copolymer polyester in which the copolymerization component is polycondensed with the main chain and/or the side chain of polyalkylene terephthalate as a main component. There are no particular limitations to the manner of polymerization and the like.

Examples of the copolymer polyester comprising polyalkylene terephthalate as a main component include a polyester obtained by copolymerizing polyethylene terephthalate as a main component with ethylene glycol ether of bisphenol A; a polyester obtained by copolymerizing polyethylene terephthalate as a main component with 1,4-cyclohexanediethanol; and a polyester obtained by copolymerizing polyethylene terephthalate as a main component with dihydroxyethyl 5-sodiumsulfoisophthalate

The polyalkylene terephthalate and its copolymer polyester may be used singly or in a combination of two or more. Preferable examples thereof include polyethylene terephthalate, polypropylene terephthalate, polybutylene terephthalate, and a copolymer polyester (a polyester obtained by copolymerizing polyethylene terephthalate as a main component with ethylene glycol ether of bisphenol A; a polyester obtained by copolymerizing polyethylene terephthalate as a main component with 1,4-cyclohexanediethanol; a polyester obtained by copolymerizing polyethylene terephthalate as a main component with dihydroxyethyl 5-sodiumsulfoisophthalate; or the like). A mixture of two or more of these is also preferable.

The component (A) has an intrinsic viscosity of preferably 0.5 to 1.4, and more preferably 0.5 to 1.0. If the intrinsic viscosity is less than 0.5, the resulting fiber tends to have reduced mechanical strength. If more than 1.4, the melt viscosity is increased as the molecular weight is increased, and thus the fiber tends to be melt spun only with difficulty, and have a non-uniform size.

There are no specific limitations to the brominated epoxy flame retardant (B) used in the present invention. A conventional brominated epoxy flame retardant may be used.

Specific examples of the component (B) include a terminal non-blocked brominated epoxy flame retardant with, containing a compound represented by the following formula (α):





20

a brominated epoxy flame retardant with one terminal blocked, containing a compound represented by the following formula ( $\beta$ ):



11

a brominated epoxy flame retardant with both terminals blocked, containing a compound represented by the following formula ( $\gamma$ ):



These may be used singly or in a combination of two or more.

The component (B) is used in an amount of 5 to 30 parts by weight based on 100 parts by weight of the component (A). In particular, the amount is preferably 6 to 25 parts by weight, and more preferably 8 to 20 parts by weight. If the component (B) is used in an amount of less than 5 parts by weight, it is difficult to achieve a flame retardant effect. If more than 30 parts by weight, mechanical properties, heat resistance, and drip resistance are impaired.

The component (B) has a number average molecular weight of preferably 20,000 or more, and more preferably 30,000 to 80,000. If the number average molecular weight is less than 20,000, a domain in which the flame retardant is dispersed in the polyester is small, projections on the fiber surface are small, and the fiber is highly glossy. If the molecular weight is too high, the dispersion domain is large, and the fiber is less colored.

As the component (C), any organic resin component may be used insofar as the component is not compatible or partially not compatible with the component (A) as a main component and/or the component (B). For example, a polyallylate, polyamide, fluororesin, silicone resin, crosslinked

12

acrylic resin, crosslinked polystyrene, and the like are preferably used. These may be used singly or in a combination of two or more.

As the component (D), such a component having a refractive index close to those of the component (A) and/or the component (B) is preferable. This is because the component 45 has an influence on transparency and coloration of the fiber. Examples include calcium carbonate, silicon oxide, titanium oxide, aluminum oxide, zinc oxide, talc, kaolin, montmorillonite, bentonite, mica, and an antimony compound. There 50 are no specific limitations to an antimony compound among these used as the component (D). Specific examples include an antimony trioxide compound, an antimony pentoxide compound, and sodium antimonite. Such an antimony compound has a particle size of preferably 0.02 to 5  $\mu\text{m}$ , more 55 preferably 0.02 to 3  $\mu\text{m}$ , and still more preferably 0.02 to 2  $\mu\text{m}$ , but the particle size is not specifically limited thereto. The antimony compound used in the present invention may be surface treated with an epoxy compound, silane compound, isocyanate compound, titanate compound, or the like as required. 60

The antimony compound is used in an amount of preferably 0.1 to 5 parts by weight, more preferably 0.1 to 3 parts by weight, and still more preferably 0.2 to 2 parts by weight based on 100 parts by weight of the component (A), but the amount is not specifically limited thereto. If the compound is used in an amount of more than 5 parts by weight, the fiber has impaired appearance, hue, and coloration. If less than 0.1 part

by weight, only a small number of minute projections are formed on the fiber surface, and thus gloss on the fiber surface is inadequately adjusted. The component (D) may be used in combination with another component (D). In this case, the components (D) are used in a total amount of 5 parts by weight.

The antimony compound is preferably used as the component (D), since the compound can not only control properties of the fiber surface, but also improve the flame retardant effect of the fiber itself.

There are no specific limitations to the hydrophilic fiber treating agent (E) used in the present invention. The fiber treating agent may be a mixture of at least one member selected from the group consisting of polyoxyalkylene alkyl ether, polyoxyalkylene alkenyl ether, polyoxyalkylene aryl ethers, and polyoxyalkylene alkylaryl ether, and their random copolymer polyethers, polyoxyalkylene alkyl ester, polyoxyalkylene alkenyl ester, and polyoxyalkylene alkylaryl ester with a conventionally used ether-containing fiber treating agent such as a polyoxyalkylene alkylamine, N,N-dihydroxyethylalkylamide, polyoxyalkylene alkylamide, glycerol fatty acid ester, polyglycerol fatty acid ester, pentaerythritol fatty acid ester, polyoxyalkylene pentaerythritol alkyl ester, sorbitan fatty acid ester, polyoxyalkylene sorbitan fatty acid ester, sucrose fatty acid ester, polyoxyalkylene sucrose fatty acid ester, polyoxyalkylene, alkylamine salt, alkylammonium salt, alkylaralkylammonium salt, alkylpyridinium salt, alkylpicolinium salt, fatty acid salt, resinate, sulfated fatty acid salt, alkyl sulfonate, alkylbenzene sulfonate, alkylnaphthalene sulfonate, sulfofatty acid alkyl ester salt, dialkyl sulfosuccinate, polyoxyalkylene alkyl ether monosulfosuccinate, polyoxyalkylene alkenyl ether monosulfosuccinate, polyoxyalkylene aryl ether monosulfosuccinate, alkyl diphenyl ether disulfonate, sulfated oil, sulfated fatty acid ester salt, alkyl sulfate, alkenyl sulfate, polyoxyalkylene alkyl ether sulfate, polyoxyalkylene alkyl ether carboxylate, polyoxyalkylene alkenyl ether sulfate, polyoxyalkylene aryl ether sulfate, alkyl phosphate, polyoxyalkylene alkyl ether phosphate, polyoxyalkylene alkenyl ether phosphate, or polyoxyalkylene aryl ether phosphate; or a mixture of a conventionally used ether-containing fiber treating agent with a conventionally used ionic surfactant. However, the fiber treating agent must not contain a compound containing a silicone component, because the treating agent has significantly reduced flame retardance if it contains a constituent having a silicone component as a main component. The hydrophilic fiber treating agent (E) is preferably at least one member selected from the group consisting of a polyether compound, fatty acid ester compound, organic amine, organic amide, organic fatty acid ester, organic amine salt, organic ammonium salt, organic pyridium salt, organic ammonium salt, organic pyridinium salt, organic picolinium salt, organic fatty acid salt, resinate, organic sulfonate, organic succinate, organic monosuccinate, organic carboxylate, and organic sulfate, or a mixture of two or more thereof, and particularly preferably at least one member selected from the group consisting of a polyethylene oxide-polypropylene oxide random copolymer polyether (molecular weight MW: 15,000 to 50,000), polyethylene oxide (molecular weight: 100 to 1,000), and polypropylene oxide (molecular weight: 100 to 1,000). The hydrophilic fiber treating agent (E) is attached to the fiber preferably at a total weight ratio of 0.01% to 1%, in order to provide smooth feeling, combing properties, antistatic properties, and the like. If the hydrophilic fiber treating agent (E) is added in an amount of 0.01% or less, the fiber has insufficient combing properties and smooth feeling. On the other hand, if 1% or more, an oil agent is attached to hands and makes the hands

wet when touching a tow filament, and the flame retardance of the fiber may be reduced since the oil agent itself is more or less flammable, unfavorably. In order to make the fiber exhibit excellent smooth feeling and combing properties and sufficient antistatic properties, a 50:50 combination of an ethylene oxide-propylene oxide random copolymer polyether with a cationic surfactant is most preferable. However, the present invention is not limited thereto. The fiber treating agent may be attached to the fiber by treatment continuous from drawing or heat treatment or by batch treatment.

The polyester fiber can have a specific modified cross-section.

When the fiber of the present invention has a cross-section in which two or more circles or flat circles are lapped or brought into contact with each other (as shown in FIGS. 1 to 3, wherein the ratio of the major axis a to the minor axis b (a/b) is 1.2 to 4), the two or more circles or flat circles lapped or brought into contact with each other are preferably arranged on a straight line and bilaterally symmetric.

When the fiber of the present invention has a cross-section with a shape of three to eight leaves (of which examples are shown in FIGS. 4 to 6, wherein the ratio of the circumscribed circle diameter D to the inscribed circle diameter d (D/d) is 1.1 to 8), the fiber has a degree of modification represented by the expression (1) of preferably 1.1 to 8, and more preferably 1.3 to 6. If the degree of modification exceeds 8, the fiber tends to exhibit impaired feeling and combing properties. If less than 1.1, the fiber tends to be felt hard. If the cross-section has a shape of nine or more leaves, its difference from a round cross-section tends to be small, and the effect of the present invention tends to be decreased.

$$\text{Degree of modification} = (\text{Circumscribed circle diameter of monofilament cross-section}) / (\text{Inscribed circle diameter of monofilament cross-section}) \quad (\text{Expression 1})$$

In the present invention, the modified cross-section has a flatness ratio (ratio of the major axis length to the minor axis length in the cross-section) of preferably 1.2 to 4, and more preferably 1.5 to 2.5, as shown in FIG. 7, wherein the ratio of the major axis x to the minor axis y (x/y) is 1.2 to 4. If the flatness ratio exceeds 4, the fiber cannot be provided with luster and feeling close to human hair. If less than 1.2, the fiber tends to have a hard texture.

When the polyester fiber of the present invention used is a mixture of a fiber having a round cross-section with a fiber having at least one modified cross-section selected from the group consisting of shapes of an ellipse, crossed circles, a cocoon, a potbelly, a dog bone, a ribbon, three to eight leaves, and a star, the mixing ratio of the fiber having a round cross-section to the fiber having a modified cross-section is preferably 8.2 to 1:9, and more preferably 7:3 to 2:8.

The modified cross-section fiber of the present invention as described above preferably has a size of 30 to 80 dtex when used for artificial hair. Further, when the modified cross-section fiber is blended with human hair at any ratio, the resulting hair goods can have any hairstyle freely. If the modified cross-section fiber of the present invention is blended in too high a proportion, the resulting product is felt hard. If the modified cross-section fiber is blended in too low a proportion, the hair goods cannot have any hairstyle freely. For this reason, it is preferable that 80 to 10 wt % of the modified cross-section fiber be blended with 20 to 80 wt % of human hair.

The modified cross-section fiber can be blended for use with another fiber for artificial hair conventionally used, for example, an acrylonitrile fiber, vinyl chloride fiber,

## 15

vinylidene chloride fiber, polyester fiber, nylon fiber, or polyolefin fiber, in addition to the aforementioned human hair.

The flame retardant polyester composition used in the present invention can be produced by, for example, dry blending the components (A) and (B) and the optional component (C) or (D) in advance, and then melt kneading the components in various common kneading machines. Examples of the kneading machines include a single-screw extruder, twin-screw extruder, roll, Banbury mixer, and kneader of these, a twin-screw extruder is preferable in terms of adjustment of the kneading degree and convenience for operation.

The flame retardant polyester fiber for artificial hair of the present invention can be produced by melt spinning the flame retardant polyester composition by a typical melt spinning process.

Specifically, a spun yarn can be obtained by, for example, melt spinning the composition while setting an extruder, gear pump, spinneret, and the like at a temperature of 270 to 310°C.; allowing the spun yarn to pass through a heating tube; then cooling the yarn to a glass transition temperature or lower; and taking off the yarn at a rate of 50 to 5,000 m/min. The size of the spun yarn can also be controlled by cooling the yarn in a tank filled with cooling water. The temperature or length of the heat sleeve, the temperature or spraying amount of cooling air, the temperature of the cooling tank, the cooling time, and the take-off rate can be appropriately adjusted according to the discharge amount and the number of holes in the spinneret.

The resulting spun yarn may be hot drawn by either a two-step process comprising winding up the spun yarn once and then drawing the yarn, or a direct spinning and drawing process comprising successively drawing the spun yarn without winding. Hot drawing is carried out by a one-stage drawing process or a multistage drawing process. As heating means in hot drawing, a heat roller, heat plate, steam jet apparatus, hot water tank, or the like can be used. These can be appropriately used in combination.

The flame retardant polyester fiber for artificial hair of the present invention may contain various additives such as a flame retardant other than the component (B), a heat resistant agent, a photostabilizer, a fluorescent agent, an antioxidant, an antistatic agent, a pigment, a plasticizer, and a lubricant as required. The fiber containing a pigment can be provided as a spun dyed fiber.

When the flame retardant polyester fiber for artificial hair of the present invention thus obtained is a fiber in the form of a non-crimped raw silk, and has a size of usually 30 to 80 dtex, and furthermore 35 to 75 dtex, the fiber is suitable for artificial hair. Preferably, the fiber for artificial hair has heat resistance to allow a thermal appliance for beauty (hair iron) to be used therefor at 160 to 200°C., catches fire only with difficulty, and has self-extinguishing properties.

When the flame retardant polyester fiber of the present invention is spun dyed, the fiber can be used as is. When the fiber is not spun dyed, it can be dyed under the same conditions as in a common flame retardant polyester fiber.

The pigment, dye, adjuvant, or the like used for dyeing preferably exhibits excellent weather resistance and flame retardance.

The flame retardant polyester fiber for artificial hair of the present invention exhibits excellent curl setting properties and curl holding properties when a thermal appliance for beauty (hair iron) is used. When the component (C) or (D) is added to the fiber if necessary, the fiber can have a surface with irregularities, can be appropriately matted, and can be more suitably used for artificial hair. Further, the hydrophilic

## 16

fiber treating agent (E) or an oil agent such as a softening agent can provide the fiber with feeling and texture and make the fiber closer to human hair.

The flame retardant polyester fiber for artificial hair of the present invention may be used in combination with another material for artificial hair such as a modacrylic fiber, polyvinyl chloride fiber, or nylon fiber, or in combination with human hair.

Generally, human hair used in hair products such as wigs, hair wigs, or extensions has cuticle treated, is bleached or dyed, and contains a silicone fiber treating agent or softening agent in order to ensure its feeling and combing properties. Thus, the human hair is flammable, unlike untreated human hair. However, when the human hair is blended with the flame retardant polyester fiber for artificial hair of the present invention at a human hair blending ratio of 60% or less, the product exhibits excellent flame retardance.

## EXAMPLES

Next, the present invention will be described in more detail with reference to Examples. However, the present invention should not be limited thereto.

Properties values are measured as follows.

## (Combing Properties)

A fiber surface treating agent is attached to a tow filament with a length of 30 cm and a total size of 100,000 dtex. The treated tow filament is combed with a comb (made of Derlin resin) to evaluate ease of combing.

Good: Filament is combed with almost no resistance (Light)

Fair: Filament is combed with a little resistance (heavy)

Bad: Filament is combed with a large resistance, or becomes uncomable in the middle

## (Strength and Elongation)

Tensile strength and elongation of a filament are measured using INTESCO Model 201 manufactured by INTESCO Co., Ltd. Both 10 mm-long ends of one 40 mm-long filament are sandwiched in a board (thin paper) to which a two-sided tape pasted with an adhesive is bonded, and are air-dried overnight to prepare a sample with a length of 20 mm. The sample is mounted on a test machine, and a test is carried out at a temperature of 24°C., at a humidity of 80% or less, at a load of 0.034 cN×size (dtex), and at a tensile rate of 20 mm/min to measure strength and elongation. The test is repeated ten times under the same conditions, and the average values are defined as strength and elongation of the filament.

## (Flame Retardance)

A filament is cut into filaments with a length of 150 mm each. Filaments with a weight of 0.7 g are bundled, with one end of the bundle sandwiched by a clamp, and the bundle is fixed on a stand and hung vertically. The fixed filaments with an effective length of 120 mm are brought into contact with 20 mm-long fire for 3 seconds, and burned.

## Flammability

Very good: Afterflame time is 0 second (Filaments do not catch fire)

Good: Afterflame time is less than 3 seconds

Fair: Afterflame time is 3 to 10 seconds

Bad: Afterflame time is more than 10 seconds

## Drip Resistance

Very good: The number of drips until extinguishment is 0

Good: The number of drips until extinguishment is 5 or less

Fair: The number of drips until extinguishment is 6 to 10

## 17

Bad: The number of drips until extinguishment is 11 or more

## (Gloss)

A tow filament with a length of 30 cm and a total size of 100,000 dtex is visually evaluated under sunlight.

Very good: Gloss is adjusted to be the same as in human hair

Good: Gloss is appropriately adjusted

Fair: Gloss is a little too high or a little too low

Bad: Gloss is too high or too low

## (Transparence)

A tow filament with a length of 30 cm and a total size of 100,000 dtex is visually evaluated under sunlight.

Good: Transparent and deep-colored (bright)

Fair: A little opaque (cloudy)

Bad: Opaque and not deep-colored

## (Devitrification Resistance)

A tow filament with a length of 10 cm and a total size of 100,000 dtex is processed with steam (at 120° C. and at a relative humidity of 100% for 1 hour), and then sufficiently dried at room temperature. The change in gloss and hue between the tow filament before steam processing and the tow filament after steam processing is examined. As the change is more significant, the tow filament exhibits lower devitrification resistance.

Very good: Neither gloss nor hue is changed

Good: Gloss is not changed, but hue is slightly changed

Fair: Both gloss and hue are slightly changed

Bad: Both gloss and hue are obviously changed

## (Feeling)

## Stickiness

A tow filament with a length of 30 cm and a total size of 100,000 dtex is allowed to stand in a room with constant temperature and humidity (at 23° C. and at a relative humidity of 55%) for 3 hours, and then evaluated using a thumb, forefinger, and middle finger on the right hand.

Good: Not sticky

Fair: A little sticky

Bad: Sticky

## Smooth Feeling

A tow filament with a length of 30 cm and a total size of 100,000 dtex is allowed to stand in a thermo-hygrostatic chamber (at 23° C. and at a relative humidity of 55%) for 3 hours, and then evaluated using a thumb, forefinger, and middle finger on the right hand.

Very good: Smooth and very slippy

Good: Smooth and slippy

Fair: Not so slippy

Bad: Not slippy

## (Surface Roughness)

Surface roughness was measured using a laser microscope (VK-9S00, manufactured by Keyence Corp.). The sides of 10 fibers in parallel with the fiber axes were measured at a

## 18

magnification of 3,000 (objective lens magnification: 150× built-in lens magnification: 20) to obtain an image. Surface roughness was calculated from this image based on a calculation formula in accordance with the definition of surface roughness (JIS B0601-1994).

## (Iron Setting Properties)

Iron setting properties are an index of the extent to which a hair iron can perform curl setting easily and hold the curl shape. Filaments are loosely sandwiched in a hair iron heated to 180° C., and pre-heated three times by rubbing. Adhesion and combing among the filaments, and frizz and breakage of the filaments are visually evaluated. Next, the pre-heated filaments are wound around the hair iron and held for 10 seconds, and then the iron is withdrawn. The degree of ease of withdrawing the iron (rod out properties) and curl holding properties when withdrawing the iron are visually evaluated.

## (Curl Setting Properties)

Straw-haired filaments are wound around a pipe with a diameter of 32 mm. Curl setting is performed at 110° C. for 60 minutes, and aging is performed at room temperature for 60 minutes. Then, one ends of the curled filaments are fixed, and the filaments are hung down to visually evaluate the degree of ease of curl setting and stability of the curl.

Good: The curl is sufficiently set and is stable

Fair: The curl is set, but is not stable

Bad: The curl is not sufficiently set

## Examples 1 to 15

To a composition made of polyethylene terephthalate dried to have a moisture content of 100 ppm or less, a brominated epoxy flame retardant, organic fine particles, and inorganic fine particles at a composition ratio shown in Tables 1 and 2, 2 parts of a coloring polyester pellet PESM6100 BLACK (manufactured by Dainichiseika Color & Chemicals Mfg. Co., Ltd., carbon black content: 30%, polyester contained in the component (A)) was added, and the components were dry blended. The blend was fed into a twin-screw extruder and melt kneaded at 280° C. to form a pellet. Then, the pellet was dried to have a moisture content of 100 ppm or less. Next, the pellet was put into a melt spinning machine, and the molten polymer was spun through a spinneret having round cross-sectional nozzle holes with a nozzle diameter of 0.5 mm each at 280° C., air-cooled, and rolled up at a rate of 100 m/min to obtain a spun yarn. The resulting spun yarn was drawn in a hot water bath at 80° C. to prepare a yarn at a draw ratio of 4. The drawn yarn was wound up around a heat roll heated to 200° C. at a rate of 30 m/min and heat-treated. Fiber treating agents KWC-Q (ethylene oxide-propylene oxide random copolymer polyether, manufactured by Marubishi Oil Chemical Co., Ltd.) and KRE-103 (cationic surfactant, manufactured by Matsumoto Yushi-Seiyaku Co., Ltd.) were attached to the yarn in an amount of 0.20 %omf, respectively, to obtain a polyester fiber (multifilament) having a monofilament size of about 50 dtex.

TABLE 1

|                       | Example |     |     |     |     |     |     |     |     |
|-----------------------|---------|-----|-----|-----|-----|-----|-----|-----|-----|
|                       | 1       | 2   | 3   | 4   | 5   | 6   | 7   | 8   | 9   |
| EFG-85A* <sup>1</sup> | 100     | 100 | 100 | 100 | 100 | 100 | 100 | 100 | 100 |
| EP-200* <sup>2</sup>  | 10      |     |     |     |     |     |     |     |     |
| EC-200* <sup>2</sup>  |         |     |     |     | 10  |     |     |     |     |

TABLE 1-continued

| Example                       |     |     |   |     |     |     |     |     |     |
|-------------------------------|-----|-----|---|-----|-----|-----|-----|-----|-----|
|                               | 1   | 2   | 3 | 4   | 5   | 6   | 7   | 8   | 9   |
| EPC-15* <sup>2</sup>          |     |     |   | 10  | 15  |     |     |     |     |
| YDB-412* <sup>3</sup>         |     |     |   |     | 10  | 15  |     |     |     |
| SR-T2000* <sup>4</sup>        |     |     |   |     |     |     | 15  |     |     |
| SR-T5000* <sup>4</sup>        |     |     |   |     |     |     |     | 10  |     |
| SR-T7040* <sup>4</sup>        |     |     |   |     |     |     |     |     | 10  |
| U Polymer U-100* <sup>5</sup> |     |     |   | 2   |     |     |     |     |     |
| Tipaque CR-60* <sup>6</sup>   | 0.2 | 0.2 |   | 0.2 |     |     |     |     |     |
| PKP-53* <sup>7</sup>          |     |     |   |     | 0.6 | 0.6 | 0.6 | 0.6 | 0.6 |

\*<sup>1</sup>Polyethylene terephthalate, manufactured by Kanebo Gohsen, Ltd.

\*2 Terminal blocked/terminal non-blocked brominated epoxy flame retardant, manufactured by Dainippon Ink and Chemicals, Inc.

\*<sup>3</sup>Terminal non-blocked brominated epoxy flame retardant, manufactured by Toho Kasei Co., Ltd.

\*<sup>4</sup>Terminal blocked/terminal non-blocked brominated epoxy flame retardant, manufactured by Sakamoto Yukihin Kogyo Co., Ltd.

\*<sup>6</sup>Titanium oxide, manufactured by Ishihara S

\*<sup>7</sup>Talc manufactured by Fujii talc Industrial Co., Ltd.

Talc, manufactured by Fuji Talc Industrial Co., Ltd.

TABLE 2

| Example                  |     |     |     |     |     |     |
|--------------------------|-----|-----|-----|-----|-----|-----|
|                          | 10  | 11  | 12  | 13  | 14  | 15  |
| EFG-85A* <sup>1</sup>    | 100 | 100 | 100 | 100 | 100 | 100 |
| XAC-4965* <sup>9</sup>   |     | 15  |     |     |     |     |
| SR-T20000* <sup>10</sup> |     |     | 12  | 16  |     |     |
| VPP-43M* <sup>11</sup>   |     |     |     |     | 5   | 10  |
|                          |     |     |     |     |     | 15  |

TABLE 2-continued

| 25                            | Example |    |     |    |    |    |
|-------------------------------|---------|----|-----|----|----|----|
|                               | 10      | 11 | 12  | 13 | 14 | 15 |
| U Polymer U-100 <sup>*5</sup> |         | 2  |     |    |    |    |
| PKP-53 <sup>*7</sup>          | 0.6     |    | 0.6 |    |    |    |

Strength and elongation, flame retardance, gloss, transparency, devitrification resistance, combing properties, feeling, surface roughness, iron setting properties, and curl setting properties of the resulting fiber were evaluated. The results are shown in Tables 3 and 4.

TABLE 2

TABLE 2-continued

|                                   |                                   | Example |      |      |      |      |      |      |      |      |
|-----------------------------------|-----------------------------------|---------|------|------|------|------|------|------|------|------|
|                                   |                                   | 1       | 2    | 3    | 4    | 5    | 6    | 7    | 8    | 9    |
| Surface roughness                 | Arithmetic mean roughness (μm)    | 0.09    | 0.09 | 0.14 | 0.07 | 0.09 | 0.09 | 0.10 | 0.11 | 0.12 |
|                                   | Ten-point mean roughness (μm)     | 0.6     | 0.7  | 1.1  | 0.5  | 0.6  | 0.7  | 0.8  | 0.8  | 0.8  |
| Iron setting properties (180° C.) | Adhesion                          | Good    | Good | Good | Good | Good | Good | Good | Good | Good |
|                                   | Crimping/end breakage             | Good    | Good | Good | Good | Good | Good | Good | Good | Good |
|                                   | Rod out                           | Good    | Good | Good | Good | Good | Good | Good | Good | Good |
| Holding properties                | Good                              | Good    | Good | Good | Good | Good | Good | Good | Good | Good |
|                                   | Curl setting properties (110° C.) | Good    | Good | Good | Good | Good | Good | Good | Good | Good |

TABLE 4

|                                                  |                                   | Example   |           |           |       |           |           |
|--------------------------------------------------|-----------------------------------|-----------|-----------|-----------|-------|-----------|-----------|
|                                                  |                                   | 10        | 11        | 12        | 13    | 14        | 15        |
| Nozzle shape                                     | Round                             | Round     | Round     | Round     | Round | Round     | Round     |
| Size (dtex)                                      | 48                                | 51        | 53        | 50        | 52    | 51        |           |
| Amount of fiber treating agents attached (% omf) | KWC-Q                             | 0.2       | 0.2       | 0.2       | 0.2   | 0.2       | 0.2       |
|                                                  | KRE-103                           | 0.2       | 0.2       | 0.2       | 0.2   | 0.2       | 0.2       |
| Strength (cN/dtex)                               | 2.6                               | 2.8       | 2.8       | 2.9       | 2.8   | 2.5       |           |
| Elongation (%)                                   | 48                                | 43        | 39        | 51        | 46    | 44        |           |
| Flame retardance                                 | Flammability                      | Very good | Very good | Very good | Good  | Good      | Very good |
|                                                  | Drip resistance                   | Very good | Very good | Very good | Good  | Very good | Very good |
| Gloss                                            | Good                              | Very good | Good      | Good      | Good  | Very good | Very good |
| Transparency                                     | Good                              | Good      | Good      | Very good | Good  | Good      | Good      |
| Devitrification resistance                       | Very good                         | Very good | Very good | Good      | Good  | Good      |           |
| Combing properties                               | Good                              | Good      | Good      | Good      | Good  | Good      |           |
| Feeling                                          | Stickiness reduction              | Good      | Good      | Good      | Good  | Good      | Good      |
|                                                  | Smooth feeling                    | Good      | Good      | Good      | Good  | Good      | Good      |
| Surface roughness                                | Arithmetic mean roughness (μm)    | 0.09      | 0.15      | 0.11      | 0.10  | 0.14      | 0.13      |
|                                                  | Ten-point mean roughness (μm)     | 0.6       | 1.1       | 0.8       | 0.7   | 1.0       | 0.8       |
| Iron setting properties (180° C.)                | Adhesion                          | Good      | Good      | Good      | Good  | Good      | Good      |
|                                                  | Crimping/end breakage             | Good      | Good      | Good      | Good  | Good      | Good      |
|                                                  | Rod out                           | Good      | Good      | Good      | Good  | Good      | Good      |
| Holding properties                               | Good                              | Good      | Good      | Good      | Good  | Good      | Good      |
|                                                  | Curl setting properties (110° C.) | Good      | Good      | Good      | Good  | Good      | Good      |

## Comparative Examples 1 to 5

To a composition made of polyethylene terephthalate dried to have a moisture content of 100 ppm or less, a brominated epoxy flame retardant, and inorganic fine particles at a composition ratio shown in Table 5, 2 parts of a coloring polyester

pellet PESM6100 BLACK (manufactured by Dainichiseika Color & Chemicals Mfg. Co., Ltd., carbon black content: 30%, polyester contained in the component (A)) was added, and the components were dry blended. The blend was fed into a twin-screw extruder and melt kneaded at 280° C. to form a pellet. Then, the pellet was dried to have a moisture content of

100 ppm or less. Next, the pellet was put into a melt spinning machine, and the molten polymer was discharged from a spinneret having round cross-sectional nozzle holes with a nozzle diameter of 0.5 mm each at 280° C., air-cooled, and wound up at a rate of 100 m/min to obtain a spun yarn. The resulting spun yarn was drawn in a hot water bath at 80° C. to prepare a yarn at a draw ratio of 4. The drawn yarn was wound up around a heat roll heated to 200° C. at a rate of 30 m/min and heat-treated. Fiber treating agents KWC-Q (ethylene oxide-propylene oxide random copolymer polyether, manufactured by Marubishi Oil Chemical Co., Ltd.) and KRE-103 (cationic surfactant, manufactured by Matsumoto Yushi-Seiyaku Co., Ltd.) were attached to the yarn in an amount of 0.20% omf, respectively, to obtain a polyester fiber (multifilament) having a monofilament size of about 50 dtex.

Strength and elongation, flame retardance, gloss, transparency, devitrification resistance, combing properties, feeling, surface roughness, iron setting properties, and curl setting properties of the resulting fiber were evaluated. The results are shown in Table 6.

TABLE 5

|                              | Comparative Example |     |    |     |     |
|------------------------------|---------------------|-----|----|-----|-----|
|                              | 1                   | 2   | 3  | 4   | 5   |
| EFG-85A* <sup>1</sup>        | 100                 | 100 |    | 100 | 100 |
| Triphenyl phosphate          | 10                  |     | 10 |     |     |
| PX-200* <sup>12</sup>        |                     |     |    | 100 |     |
| Heim RH-416* <sup>13</sup>   |                     |     |    |     | 100 |
| Pyrochek 68PB* <sup>14</sup> |                     |     |    |     | 6   |
| FR-1808* <sup>15</sup>       |                     |     |    |     | 10  |
| Tipaque CR-60* <sup>6</sup>  |                     |     | 1  |     |     |

\*<sup>1</sup>Polyethylene terephthalate, manufactured by Kanebo Gohsen, Ltd.

\*<sup>12</sup>Condensed phosphate flame retardant, manufactured by Daihachi Chemical Industry Co., Ltd.

\*<sup>13</sup>Phosphorus flame retardant copolymer polyester, manufactured by Toyobo Co., Ltd.

\*<sup>14</sup>Brominated polystyrene flame retardant, manufactured by Nissan Ferro Organic Chemical Co., Ltd.

\*<sup>15</sup>Octabromotrimethylphenylindane, manufactured by Bromokem Far East Ltd.

\*<sup>6</sup>Titanium oxide, manufactured by Ishihara Sangyo Kaisha, Ltd.

TABLE 6

|                                                  | Comparative Example               |                |       |       |              |
|--------------------------------------------------|-----------------------------------|----------------|-------|-------|--------------|
|                                                  | 1                                 | 2              | 3     | 4     | 5            |
| Nozzle shape                                     | Round                             | Round          | Round | Round | Round        |
| Size (dtex)                                      | 52                                | 48             | 47    | 47    | 50           |
| Amount of fiber treating agents attached (% omf) | KWC-Q<br>0.2                      | KRE-103<br>0.2 |       | 0.2   | 0.2          |
| Strength (cN/dtex)                               | 2.2                               | 2.0            | 1.9   | 2.9   | 2.6          |
| Elongation (%)                                   | 68                                | 63             | 42    | 52    | 47           |
| Flame retardance                                 | Flammability                      | Fair           | Fair  | Good  | Very<br>good |
|                                                  | Drip resistance                   | Bad            | Bad   | Bad   | Very<br>good |
| Gloss                                            |                                   | Bad            | Fair  | Fair  | Very<br>good |
| Transparency                                     |                                   | Fair           | Fair  | Fair  | Bad          |
| Devitrification resistance                       |                                   | Fair           | Fair  | Bad   | Fair         |
| Combing properties                               |                                   | Bad            | Bad   | Fair  | Bad          |
| Feeling                                          | Stickiness<br>reduction           | Bad            | Bad   | Bad   | good         |
|                                                  | Smooth feeling                    | Bad            | Bad   | Bad   | Bad          |
| Surface roughness                                | Arithmetic mean<br>roughness (μm) | 0.01           | 0.06  | 0.05  | 0.12         |
|                                                  | Ten point mean<br>roughness (μm)  | 0.1            | 0.4   | 0.4   | 0.5          |
| Iron setting properties<br>(180° C.)             | Adhesion                          | Bad            | Bad   | Good  | Good         |
|                                                  | Crimping/end<br>breakage          | Fair           | Fair  | Fair  | Good         |
|                                                  | Rod out                           | Bad            | Bad   | Bad   | Good         |
| Holding properties                               | Good                              | Good           | Good  | Good  | Good         |
| Curl setting properties<br>(110° C.)             |                                   | Fair           | Fair  | Fair  | Fair         |

As shown in Tables 3 and 4, it was confirmed that the fibers of Examples are superior to the fibers of Comparative Examples in terms of flame retardance, gloss, transparency, devitrification resistance, combing properties, feeling, iron setting properties, and curl setting properties. Accordingly, it was confirmed that the fiber for artificial hair of interest using a brominated epoxy flame retardant can be effectively used as artificial hair with improved flame retardance, gloss, transparency, setting properties, devitrification resistance, and combing properties, while maintaining mechanical properties and thermal properties possessed by polyester.

### Examples 16 to 22

To a composition made of polyethylene terephthalate dried to have a moisture content of 100 ppm or less, a brominated epoxy flame retardant, and inorganic fine particles at a composition ratio shown in Table 7, 2 parts of a coloring polyester pellet PESM6100 BLACK (manufactured by Dainichiseika Color & Chemicals Mfg. Co., Ltd., carbon black content: 30%, polyester contained in the component (A)) was added, and the components were dry blended. The blend was fed into a twin-screw extruder and melt kneaded at 280°C. to form a pellet. Then, the pellet was dried to have a moisture content of 100 ppm or less. Next, the pellet was put into a melt spinning machine, and the molten polymer was discharged from a spinneret having nozzle holes with a cross-section of FIGS. 8 to 10 at 280°C., air-cooled, and wound up at a rate of 100 m/min to obtain a spun yarn. The resulting spun yarn was drawn in a hot water bath at 80°C. to prepare a yarn at a draw ratio of 4. The drawn yarn was wound up around a heat roll heated to 200°C. at a rate of 30 m/min and heat-treated. Fiber treating agents KWC-Q (ethylene oxide-propylene oxide ran-

dom copolymer polyether, manufactured by Marubishi Oil Chemical Co., Ltd.) and KRE-103 (cationic surfactant, manufactured by Matsumoto Yushi-Seiyaku Co., Ltd.) were attached to the yarn in an amount of 0.20% omf, respectively, to obtain a polyester fiber (multifilament) having a monofilament size of about 60 to 70 dtex.

TABLE 7

| 10                       |     | Example |     |     |     |     |     |     |
|--------------------------|-----|---------|-----|-----|-----|-----|-----|-----|
|                          |     | 16      | 17  | 18  | 19  | 20  | 21  | 22  |
| EFG-85A* <sup>1</sup>    | 100 | 100     | 100 | 100 | 100 | 100 | 100 | 100 |
| SR-T20000* <sup>10</sup> | 10  | 10      | 10  | 10  | 10  | 10  | 15  | 15  |
| YPB-43M* <sup>11</sup>   |     |         |     |     |     |     |     |     |
| PKP-53* <sup>7</sup>     | 0.5 | 0.5     | 0.5 | 0.5 | 0.5 | 0.5 |     |     |
| Imsil A-8* <sup>16</sup> | 0.5 | 0.5     | 0.5 | 0.5 | 0.5 | 0.5 |     |     |

\*<sup>1</sup>Polyethylene terephthalate, manufactured by Kanebo Gohsen, Ltd.

\*<sup>10</sup>Terminal non-blocked brominated epoxy flame retardant, number average molecular weight: 30,000, manufactured by Sakamoto Yakuhan Kogyo Co., Ltd.

\*<sup>11</sup>Terminal non-blocked brominated epoxy flame retardant, number average molecular weight: 40,000, manufactured by Tohco Kasei Co., Ltd.

\*<sup>7</sup>Talc, manufactured by Fuji talc Industrial Co., Ltd.

\*<sup>16</sup>Silica, manufactured by Unimin Corp.

(In FIG. 8, A is 0.9 mm, and B is 0.4 mm.)

25 (In FIG. 9, A is 1.0 mm, B is 0.35 mm, and C is 0.25 mm.)

(In FIG. 10, R is 0.6 mm, and r is 0.4 mm.)

Strength and elongation, flame retardance, gloss, transparency, devitrification resistance, combing properties, feeling, surface roughness, iron setting properties, and curl setting properties of the resulting fiber were evaluated. The results are shown in Table 8.

TABLE 8

| Nozzle shape               | Example                          |           |           |           |           |           |           |
|----------------------------|----------------------------------|-----------|-----------|-----------|-----------|-----------|-----------|
|                            | 16                               | 17        | 18        | 19        | 20        | 21        | 22        |
| Size (dtex)                | 67                               | 65        | 68        | 62        | 59        | 70        | 68        |
| Amount of fiber            | 0.2                              | 0.2       | 0.2       | 0.2       | 0.2       | 0.2       | 0.2       |
| treating agents attached   |                                  |           |           |           |           |           |           |
| (% omf)                    |                                  |           |           |           |           |           |           |
| Strength (cN/dtex)         | 2.5                              | 2.2       | 1.8       | 2.7       | 2.9       | 2.4       | 2.2       |
| Elongation (%)             | 68                               | 53        | 38        | 59        | 52        | 53        | 48        |
| Flame retardance           | Very good                        | Very good | Very good | Very good | Very good | Very good | Very good |
| Drip resistance            | Very good                        | Very good | Very good | Very good | Very good | Very good | Very good |
| Gloss                      | Good                             | Good      | Good      | Good      | Good      | Very good | Very good |
| Transparency               | Good                             | Good      | Good      | Good      | Good      | Good      | Good      |
| Devitrification resistance | Good                             | Good      | Good      | Good      | Good      | Good      | Good      |
| Combing properties         | Good                             | Good      | Good      | Good      | Good      | Good      | Good      |
| Feeling                    | Good                             | Good      | Good      | Good      | Good      | Good      | Good      |
| reduction                  |                                  |           |           |           |           |           |           |
| Smooth feeling             | Very good                        | Very good | Very good | Very good | Very good | Very good | Very good |
| Surface roughness          | Arithmetic mean roughness (μm)   | 1.0       | 1.0       | 1.1       | 1.0       | 1.1       | 1.4       |
|                            | Ten-point surface roughness (μm) | 0.8       | 0.9       | 0.8       | 0.7       | 0.8       | 1.1       |

TABLE 8-continued

| Example                           |                                 |           |           |           |           |           |           |
|-----------------------------------|---------------------------------|-----------|-----------|-----------|-----------|-----------|-----------|
|                                   | 16                              | 17        | 18        | 19        | 20        | 21        | 22        |
| Iron setting properties (180° C.) | Adhesion Crimping/ end breakage | Good Good | Good Good | Good Good | Good Good | Good Good | Good Good |
|                                   | Rod out Holding properties      | Good Good | Good Good | Good Good | Good Good | Good Good | Good Good |
| Curl setting properties (110° C.) | Good                            | Good      | Good      | Good      | Good      | Good      | Good      |

15

## Examples 23 to 29

To a composition made of polyethylene terephthalate dried to have a moisture content of 100 ppm or less, a brominated epoxy flame retardant, and inorganic fine particles at a composition ratio shown in Table 9, 2 parts of a coloring polyester pellet PESM6100 BLACK (manufactured by Dainichiseika Color & Chemicals Mfg. Co., Ltd., carbon black content: 30%, polyester contained in the component (A)) was added, and the components were dry blended. The blend was fed into a twin-screw extruder and melt kneaded at 280° C. to form a pellet. Then, the pellet was dried to have a moisture content of 100 ppm or less. Next, the pellet was put into a melt spinning machine, and the molten polymer was spun through a spinneret having nozzle holes with a cross-section of FIGS. 8 and 9 at 280° C., air-cooled, and rolled up at a rate of 100 m/min to obtain a spun yarn. The resulting spun yarn was drawn in a hot water bath at 80° C. to prepare a yarn at a draw ratio of 4. The drawn yarn was rolled up around a heat roll heated to 200° C. at a rate of 30 m/min and heat-treated. Fiber treating

agents shown in Table 10 were respectively attached to the yarn to obtain a polyester fiber (multifilament) having a monofilament size of about 70 dtex.

TABLE 9

|                          | Example |     |     |     |     |     |     |
|--------------------------|---------|-----|-----|-----|-----|-----|-----|
|                          | 23      | 24  | 25  | 26  | 27  | 28  | 29  |
| EFG-85A* <sup>1</sup>    | 100     | 100 | 100 | 100 | 100 | 100 | 100 |
| SR-T20000* <sup>10</sup> | 16      | 16  | 16  | 16  | 16  |     |     |
| YPB-43M* <sup>11</sup>   |         |     |     |     |     | 15  | 15  |
| PKP-53* <sup>7</sup>     | 0.6     | 0.6 | 0.6 | 0.6 | 0.6 |     |     |

30 \*<sup>1</sup>Polyethylene terephthalate, manufactured by Kanebo Gohsen, Ltd.

\*<sup>10</sup>Terminal non-blocked brominated epoxy flame retardant, number average molecular weight: 30,000, manufactured by Sakamoto Yakuhin Kogyo Co., Ltd.

\*<sup>11</sup>Terminal non-blocked brominated epoxy flame retardant, number average molecular weight: 40,000, manufactured by Tohoku Kasei Co., Ltd.

\*<sup>7</sup>Talc, manufactured by Fuji Talc Industrial Co., Ltd.

TABLE 10

| Example                    |                                                |            |            |            |            |            |            |
|----------------------------|------------------------------------------------|------------|------------|------------|------------|------------|------------|
|                            | 23                                             | 24         | 25         | 26         | 27         | 28         | 29         |
| Nozzle shape               | Modified 1                                     | Modified 1 | Modified 1 | Modified 1 | Modified 1 | Modified 2 | Modified 2 |
| Size (dtex)                | 70                                             | 70         | 70         | 70         | 70         | 68         | 68         |
| Amount of fiber            | KWC-Q* <sup>17</sup><br>KRE-103* <sup>18</sup> | 0.1<br>0.1 | 0.25       | 0.15       |            | 0.1<br>0.1 |            |
| treating agents            | KRE-102* <sup>19</sup>                         |            | 0.2        | 0.1        |            |            |            |
| attached agents            | KRE-15* <sup>20</sup>                          |            |            |            | 0.2        | 0.1        | 0.1        |
| attached agents            | KRE-16* <sup>21</sup>                          |            |            |            | 0.14       | 0.07       | 0.07       |
| (% omf)                    | KRE-17* <sup>22</sup>                          |            |            |            | 0.06       | 0.03       | 0.03       |
| Strength (cN/dtex)         | 2.5                                            | 2.5        | 2.5        | 2.5        | 2.5        | 2.4        | 2.4        |
| Elongation (%)             | 54                                             | 54         | 54         | 54         | 54         | 48         | 48         |
| Flame retardance           | Very good                                      | Very good  | Very good  | Very good  | Very good  | Very good  | Very good  |
| Drip resistance            | Very good                                      | Very good  | Very good  | Very good  | Very good  | Very good  | Very good  |
| Gloss                      | Good                                           | Good       | Good       | Good       | Good       | Very good  | Very good  |
| Transparency               | Good                                           | Good       | Good       | Good       | Good       | Good       | Good       |
| Devitrification resistance | Good                                           | Good       | Good       | Good       | Good       | Good       | Good       |
| Combing properties         | Good                                           | Good       | Good       | Good       | Good       | Good       | Good       |
| Feeling                    | Stickiness reduction                           | Good       | Good       | Good       | Good       | Good       | Good       |
|                            | Smooth feeling                                 | Good       | Very good  | Good       | Very good  | Good       | Good       |
| Surface roughness          | Arithmetic surface roughness (μm)              | 1.0        | 1.0        | 1.0        | 1.0        | 1.4        | 1.4        |
|                            | Ten-point surface roughness (μm)               | 0.8        | 0.8        | 0.8        | 0.8        | 1.1        | 1.1        |

TABLE 10-continued

|                                   |                                 | Example   |           |           |           |           |           |           |
|-----------------------------------|---------------------------------|-----------|-----------|-----------|-----------|-----------|-----------|-----------|
|                                   |                                 | 23        | 24        | 25        | 26        | 27        | 28        | 29        |
| Iron setting properties (180° C.) | Adhesion Crimping/ end breakage | Good Good | Good Good | Good Good | Good Good | Good Good | Good Good | Good Good |
|                                   | Rod out Holding properties      | Good Good | Good Good | Good Good | Good Good | Good Good | Good Good | Good Good |
| Curl setting properties (110° C.) |                                 | Good      | Good      | Good      | Good      | Good      | Good      | Good      |

15

As shown in Tables 8 and 10, it was confirmed that a fiber for artificial hair having excellent properties and quality balance can be obtained by modifying the fiber cross-section or using a specific fiber treating agent.

#### INDUSTRIAL APPLICABILITY

An object of the present invention is to provide a flame retardant polyester fiber for artificial hair in which problems of the prior art are solved and which maintains fiber properties such as heat resistance and strength and elongation possessed by a common polyester fiber, has excellent flame retardance, setting properties, drip resistance, transparency, devitrification resistance, stickiness reduction, and combing properties required for artificial hair, and has fiber luster controlled according to need.

Another object of the present invention is to provide a polyester fiber for artificial hair which maintains fiber properties such as heat resistance and strength and elongation possessed by a polyester fiber, improves defective curling properties of such a polyester fiber, and has excellent luster, feeling, and combing properties by using the above-described polyester fiber for artificial hair which has at least one modified cross-section, is a mixture with a fiber having a modified cross-section, and has a mixing ratio of the fiber having a round cross-section to the fiber having a modified cross-section is 8:2 to 1:9.

The present invention further provides a flame retardant fiber for artificial hair which does not have reduced flame retardance as in the case where such a fiber is treated with a silicone fiber treating agent in order to improve smooth feeling and texture, for example; has slip feeling and combing properties the same as in the case where such a fiber is treated with a silicone oil agent for the same purpose; and has excellent flame retardance.

The invention claimed is:

1. A flame retardant polyester artificial hair, comprising 100 parts by weight of (A) a polyester made of one or more of 20 polyalkylene terephthalate or copolymer polyester, which comprises polyalkylene terephthalate as a main component, and 5 to 30 parts by weight of (B) a brominated epoxy flame retardant represented by the following general formula (1):



30 wherein m represents 30 to 150, and having a monofilament size of 30 to 80 dtex.

35 40 45 50 55 60 65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000 1005 1010 1015 1020 1025 1030 1035 1040 1045 1050 1055 1060 1065 1070 1075 1080 1085 1090 1095 1100 1105 1110 1115 1120 1125 1130 1135 1140 1145 1150 1155 1160 1165 1170 1175 1180 1185 1190 1195 1200 1205 1210 1215 1220 1225 1230 1235 1240 1245 1250 1255 1260 1265 1270 1275 1280 1285 1290 1295 1300 1305 1310 1315 1320 1325 1330 1335 1340 1345 1350 1355 1360 1365 1370 1375 1380 1385 1390 1395 1400 1405 1410 1415 1420 1425 1430 1435 1440 1445 1450 1455 1460 1465 1470 1475 1480 1485 1490 1495 1500 1505 1510 1515 1520 1525 1530 1535 1540 1545 1550 1555 1560 1565 1570 1575 1580 1585 1590 1595 1600 1605 1610 1615 1620 1625 1630 1635 1640 1645 1650 1655 1660 1665 1670 1675 1680 1685 1690 1695 1700 1705 1710 1715 1720 1725 1730 1735 1740 1745 1750 1755 1760 1765 1770 1775 1780 1785 1790 1795 1800 1805 1810 1815 1820 1825 1830 1835 1840 1845 1850 1855 1860 1865 1870 1875 1880 1885 1890 1895 1900 1905 1910 1915 1920 1925 1930 1935 1940 1945 1950 1955 1960 1965 1970 1975 1980 1985 1990 1995 2000 2005 2010 2015 2020 2025 2030 2035 2040 2045 2050 2055 2060 2065 2070 2075 2080 2085 2090 2095 2100 2105 2110 2115 2120 2125 2130 2135 2140 2145 2150 2155 2160 2165 2170 2175 2180 2185 2190 2195 2200 2205 2210 2215 2220 2225 2230 2235 2240 2245 2250 2255 2260 2265 2270 2275 2280 2285 2290 2295 2300 2305 2310 2315 2320 2325 2330 2335 2340 2345 2350 2355 2360 2365 2370 2375 2380 2385 2390 2395 2400 2405 2410 2415 2420 2425 2430 2435 2440 2445 2450 2455 2460 2465 2470 2475 2480 2485 2490 2495 2500 2505 2510 2515 2520 2525 2530 2535 2540 2545 2550 2555 2560 2565 2570 2575 2580 2585 2590 2595 2600 2605 2610 2615 2620 2625 2630 2635 2640 2645 2650 2655 2660 2665 2670 2675 2680 2685 2690 2695 2700 2705 2710 2715 2720 2725 2730 2735 2740 2745 2750 2755 2760 2765 2770 2775 2780 2785 2790 2795 2800 2805 2810 2815 2820 2825 2830 2835 2840 2845 2850 2855 2860 2865 2870 2875 2880 2885 2890 2895 2900 2905 2910 2915 2920 2925 2930 2935 2940 2945 2950 2955 2960 2965 2970 2975 2980 2985 2990 2995 3000 3005 3010 3015 3020 3025 3030 3035 3040 3045 3050 3055 3060 3065 3070 3075 3080 3085 3090 3095 3100 3105 3110 3115 3120 3125 3130 3135 3140 3145 3150 3155 3160 3165 3170 3175 3180 3185 3190 3195 3200 3205 3210 3215 3220 3225 3230 3235 3240 3245 3250 3255 3260 3265 3270 3275 3280 3285 3290 3295 3300 3305 3310 3315 3320 3325 3330 3335 3340 3345 3350 3355 3360 3365 3370 3375 3380 3385 3390 3395 3400 3405 3410 3415 3420 3425 3430 3435 3440 3445 3450 3455 3460 3465 3470 3475 3480 3485 3490 3495 3500 3505 3510 3515 3520 3525 3530 3535 3540 3545 3550 3555 3560 3565 3570 3575 3580 3585 3590 3595 3600 3605 3610 3615 3620 3625 3630 3635 3640 3645 3650 3655 3660 3665 3670 3675 3680 3685 3690 3695 3700 3705 3710 3715 3720 3725 3730 3735 3740 3745 3750 3755 3760 3765 3770 3775 3780 3785 3790 3795 3800 3805 3810 3815 3820 3825 3830 3835 3840 3845 3850 3855 3860 3865 3870 3875 3880 3885 3890 3895 3900 3905 3910 3915 3920 3925 3930 3935 3940 3945 3950 3955 3960 3965 3970 3975 3980 3985 3990 3995 4000 4005 4010 4015 4020 4025 4030 4035 4040 4045 4050 4055 4060 4065 4070 4075 4080 4085 4090 4095 4100 4105 4110 4115 4120 4125 4130 4135 4140 4145 4150 4155 4160 4165 4170 4175 4180 4185 4190 4195 4200 4205 4210 4215 4220 4225 4230 4235 4240 4245 4250 4255 4260 4265 4270 4275 4280 4285 4290 4295 4300 4305 4310 4315 4320 4325 4330 4335 4340 4345 4350 4355 4360 4365 4370 4375 4380 4385 4390 4395 4400 4405 4410 4415 4420 4425 4430 4435 4440 4445 4450 4455 4460 4465 4470 4475 4480 4485 4490 4495 4500 4505 4510 4515 4520 4525 4530 4535 4540 4545 4550 4555 4560 4565 4570 4575 4580 4585 4590 4595 4600 4605 4610 4615 4620 4625 4630 4635 4640 4645 4650 4655 4660 4665 4670 4675 4680 4685 4690 4695 4700 4705 4710 4715 4720 4725 4730 4735 4740 4745 4750 4755 4760 4765 4770 4775 4780 4785 4790 4795 4800 4805 4810 4815 4820 4825 4830 4835 4840 4845 4850 4855 4860 4865 4870 4875 4880 4885 4890 4895 4900 4905 4910 4915 4920 4925 4930 4935 4940 4945 4950 4955 4960 4965 4970 4975 4980 4985 4990 4995 5000 5005 5010 5015 5020 5025 5030 5035 5040 5045 5050 5055 5060 5065 5070 5075 5080 5085 5090 5095 5100 5105 5110 5115 5120 5125 5130 5135 5140 5145 5150 5155 5160 5165 5170 5175 5180 5185 5190 5195 5200 5205 5210 5215 5220 5225 5230 5235 5240 5245 5250 5255 5260 5265 5270 5275 5280 5285 5290 5295 5300 5305 5310 5315 5320 5325 5330 5335 5340 5345 5350 5355 5360 5365 5370 5375 5380 5385 5390 5395 5400 5405 5410 5415 5420 5425 5430 5435 5440 5445 5450 5455 5460 5465 5470 5475 5480 5485 5490 5495 5500 5505 5510 5515 5520 5525 5530 5535 5540 5545 5550 5555 5560 5565 5570 5575 5580 5585 5590 5595 5600 5605 5610 5615 5620 5625 5630 5635 5640 5645 5650 5655 5660 5665 5670 5675 5680 5685 5690 5695 5700 5705 5710 5715 5720 5725 5730 5735 5740 5745 5750 5755 5760 5765 5770 5775 5780 5785 5790 5795 5800 5805 5810 5815 5820 5825 5830 5835 5840 5845 5850 5855 5860 5865 5870 5875 5880 5885 5890 5895 5900 5905 5910 5915 5920 5925 5930 5935 5940 5945 5950 5955 5960 5965 5970 5975 5980 5985 5990 5995 6000 6005 6010 6015 6020 6025 6030 6035 6040 6045 6050 6055 6060 6065 6070 6075 6080 6085 6090 6095 6100 6105 6110 6115 6120 6125 6130 6135 6140 6145 6150 6155 6160 6165 6170 6175 6180 6185 6190 6195 6200 6205 6210 6215 6220 6225 6230 6235 6240 6245 6250 6255 6260 6265 6270 6275 6280 6285 6290 6295 6300 6305 6310 6315 6320 6325 6330 6335 6340 6345 6350 6355 6360 6365 6370 6375 6380 6385 6390 6395 6400 6405 6410 6415 6420 6425 6430 6435 6440 6445 6450 6455 6460 6465 6470 6475 6480 6485 6490 6495 6500 6505 6510 6515 6520 6525 6530 6535 6540 6545 6550 6555 6560 6565 6570 6575 6580 6585 6590 6595 6600 6605 6610 6615 6620 6625 6630 6635 6640 6645 6650 6655 6660 6665 6670 6675 6680 6685 6690 6695 6700 6705 6710 6715 6720 6725 6730 6735 6740 6745 6750 6755 6760 6765 6770 6775 6780 6785 6790 6795 6800 6805 6810 6815 6820 6825 6830 6835 6840 6845 6850 6855 6860 6865 6870 6875 6880 6885 6890 6895 6900 6905 6910 6915 6920 6925 6930 6935 6940 6945 6950 6955 6960 6965 6970 6975 6980 6985 6990 6995 7000 7005 7010 7015 7020 7025 7030 7035 7040 7045 7050 7055 7060 7065 7070 7075 7080 7085 7090 7095 7100 7105 7110 7115 7120 7125 7130 7135 7140 7145 7150 7155 7160 7165 7170 7175 7180 7185 7190 7195 7200 7205 7210 7215 7220 7225 7230 7235 7240 7245 7250 7255 7260 7265 7270 7275 7280 7285 7290 7295 7300 7305 7310 7315 7320 7325 7330 7335 7340 7345 7350 7355 7360 7365 7370 7375 7380 7385 7390 7395 7400 7405 7410 7415 7420 7425 7430 7435 7440 7445 7450 7455 7460 7465 7470 7475 7480 7485 7490 7495 7500 7505 7510 7515 7520 7525 7530 7535 7540 7545 7550 7555 7560 7565 7570 7575 7580 7585 7590 7595 7600 7605 7610 7615 7620 7625 7630 7635 7640 7645 7650 7655 7660 7665 7670 7675 7680 7685 7690 7695 7700 7705 7710 7715 7720 7725 7730 7735 7740 7745 7750 7755 7760 7765 7770 7775 7780 7785 7790 7795 7800 7805 7810 7815 7820 7825 7830 7835 7840 7845 7850 7855 7860 7865 7870 7875 7880 7885 7890 7895 7900 7905 7910 7915 7920 7925 7930 7935 7940 7945 7950 7955 7960 7965 7970 7975 7980 7985 7990 7995 8000 8005 8010 8015 8020 8025 8030 8035 8040 8045 8050 8055 8060 8065 8070 8075 8080 8085 8090 8095 8100 8105 8110 8115 8120 8125 8130 8135 8140 8145 8150 8155 8160 8165 8170 8175 8180 8185 8190 8195 8200 8205 8210 8215 8220 8225 8230 8235 8240 8245 8250 8255 8260 8265 8270 8275 8280 8285 8290 8295 8300 8305 8310 8315 8320 8325 8330 8335 8340 8345 8350 8355 8360 8365 8370 8375 8380 8385 8390 8395 8400 8405 8410 8415 8420 8425 8430 8435 8440 8445 8450 8455 8460 8465 8470 8475 8480 8485 8490 8495 8500 8505 8510 8515 8520 8525 8530 8535 8540 8545 8550 8555 8560 8565 8570 8575 8580 8585 8590 8595 8600 8605 8610 8615 8620 8625 8630 8635 8640 8645 8650 8655 8660 8665 8670 8675 8680 8685 8690 8695 8700 8705 8710 8715 8720 8725 8730 8735 8740 8745 8750 8755 8760 8765 8770 8775 8780 8785 8790 8795 8800 8805 8810 8815 8820 8825 8830 8835 8840 8845 8850 8855 8860 8865 8870 8875 8880 8885 8890 8895 8900 8905 8910 8915 8920 8925 8930 8935 8940 8945 8950 8955 8960 8965 8970 8975 8980 8985 8990 8995 9000 9005 9010 9015 9020 9025 9030 9035 9040 9045 9050 9055 9060 9065 9070 9075 9080 9085 9090 9095 9100 9105 9110 9115 9120 9125 9130 9135 9140 9145 9150 9155 9160 9165 9170 9175 9180 9185 9190 9195 9200 9205 9210 9215 9220 9225 9230 9235 9240 9245 9250 9255 9260 9265 9270 9275 9280 9285 9290 9295 9300 9305 9310 9315 9320 9325 9330 9335 9340 9345 9350 9355 9360 9365 9370 9375 9380 9385 9390 9395 9400 9405 9410 9415 9420 9425 9430 9435 9440 9445 9450 9455 9460 9465 9470 9475 9480 9485 9490 9495 9500 9505 9510 9515 9520 9525 9530 9535 9540 9545 9550 9555 9560 9565 9570 9575 9580 9585 9590 9595 9600 9605 9610 9615 9620 9625 9630 9635 9640 9645 9650 9655 9660 9665 9670 9675 9680 9685 9690 9695 9700 9705 9710 9715 9720 9725 9730 9735 9740 9745 9750 9755 9760 9765 9770 9775 9780 9785 9790 9795 9800 9805 9810 9815 9820 9825 9830 9835 9840 98

31

wherein m represents 30 to 150,

32



wherein  $R^1$  represents a  $C_{1-10}$  alkyl group, n represents 30 to 100, and y represents 0 to 4,

(7)



wherein  $R^1$  represents a  $C_{1-10}$  alkyl group, n represents 30 to 100, and y represents 0 to 4.

5. The flame retardant polyester artificial hair according to claim 2 or 3, wherein the hair surface has amorphous projections.

6. The flame retardant polyester artificial hair according to claim 2 or 3, wherein the hair surface has projections which have a major axis length of 0.2 to 20  $\mu m$ , a minor axis length of 0.1 to 10  $\mu m$ , and a height of 0.1 to 2  $\mu m$ , respectively.

7. The flame retardant polyester artificial hair according to claim 1, 2, or 3, which is formed from a composition obtained by further mixing the components (A) and (B) with at least one selected from the group consisting of organic fine particles (C) and inorganic fine particles (D), and has minute projections on the hair surface.

8. The flame retardant polyester artificial hair according to claim 7, wherein the component (C) is at least one member selected from the group consisting of a polyarylate, polyamide, fluororesin, silicone resin, crosslinked acrylic resin, and crosslinked polystyrene.

9. The flame retardant polyester artificial hair according to claim 7, wherein the component (D) is at least one member selected from the group consisting of calcium carbonate, silicon oxide, titanium oxide, aluminum oxide, zinc oxide, talc, kaolin, montmorillonite, bentonite, and mica.

10. The flame retardant polyester artificial hair according to claim 1, 2, or 3, which has at least one modified cross-section selected from the group consisting of shapes of an ellipse, crossed circles, a cocoon, a potbelly, a dog bone, a ribbon, three to eight leaves, and a star.

11. The flame retardant polyester artificial hair according to claim 10, wherein the hair cross-section has a shape with two or more circles or flat circles lapped or brought into contact with each other.

12. The flame retardant polyester artificial hair according to claim 10, wherein the hair cross-section has a shape of three to eight leaves, and the hair is a modified cross-section hair having a degree of modification represented by the expression (1) of 1.1 to 8

Degree of modification = (Circumscribed circle diameter of monofilament cross-section) / (Inscribed circle diameter of monofilament cross-section) (Expression 1).

13. The flame retardant polyester artificial hair according to claim 10, wherein the hair cross-section has a flatness ratio of 1.2 to 4.

14. The flame retardant polyester artificial hair according to claim 10, which is a mixture of a hair having a round cross-section with a hair having at least one modified cross-section selected from the group consisting of shapes of an ellipse, crossed circles, a cocoon, a potbelly, a dog bone, a ribbon, three to eight leaves, and a star, wherein the mixing ratio of the hair having a round cross-section to the hair having a modified cross-section is 8:2 to 1:9.

15. The flame retardant polyester artificial hair according to claim 1, 2, or 3, further comprising (E) a hydrophilic fiber treating agent attached thereto.

16. The flame retardant polyester artificial hair according to claim 15, wherein the component (E) is at least one member selected from the group consisting of a polyether compound,

33

fatty acid ester compound, organic amine, organic amide, organic fatty acid ester, organic amine salt, organic ammonium salt, organic pyridinium salt, organic ammonium salt, organic pyridinium salt, organic picolinium salt, organic fatty acid salt, resinate, organic sulfonate, organic succinate, organic monosuccinate, organic carboxylate, organic sulfate, and organic phosphate.

17. The flame retardant polyester artificial hair according to claim 1 or 2, wherein the component (E) is at least one member selected from the group consisting of polyoxyalkylene alkyl ether, polyoxyalkylene alkenyl ether, and polyoxyalkylene aryl ether, and their random copolymer polyethers, polyoxyalkylene alkylaryl ether, polyoxyalkylene alkyl ester, polyoxyalkylene alkenyl ester, and polyoxyalkylene alkylaryl ester.

34

18. The flame retardant polyester artificial hair according to claim 15, wherein the component (E) is at least one member selected from the group consisting of an ethylene oxide-propylene oxide random copolymer polyether (molecular weight MW: 15,000 to 50,000), polyethylene oxide (molecular weight: 100 to 1,000), and polypropylene oxide (molecular weight: 100 to 1,000).

19. The flame retardant polyester artificial hair according to claim 18, wherein the component (E) is attached to the hair at a weight ratio of 0.01% to 1%.

20. The flame retardant polyester artificial hair according to claim 1, 2, or 3, which is in the form of a non-crimped raw silk.

21. The flame retardant polyester artificial hair according to claim 1, 2, or 3, which is spun dyed hair.

\* \* \* \* \*